

# United States Patent

[11] 3,603,792

[72] Inventors Anthony V. Gallaro  
 Auburn, N.Y.;  
 Walter F. Kazuk, Loves Park, Ill.; Kenneth  
 Speigel, Seneca Falls, N.Y.  
 [21] Appl. No. 853,085  
 [22] Filed Aug. 26, 1969  
 Division of Ser. No. 634,724, Apr. 28, 1967,  
 Pat. No. 3,526,527  
 [45] Patented Sept. 7, 1971  
 [73] Assignee GT & E Sylvania Incorporated

[56] References Cited  
 UNITED STATES PATENTS  
 2,798,823 7/1957 Harper ..... 250/80 X  
 2,835,822 5/1958 Williams ..... 250/80  
 3,046,154 6/1962 Feldman ..... 250/80 X  
 Primary Examiner—James W. Lawrence  
 Assistant Examiner—Davis L. Willis  
 Attorneys—Norman J. O'Malley, Donald R. Castle and  
 Frederick H. Rinn

[54] LUMINESCENT SCREEN HAVING A SEPARATION  
 MEDIUM THEREIN  
 3 Claims, 3 Drawing Figs.  
 [52] U.S. Cl. 250/80, 313/92 PH  
 [51] Int. Cl. H01j 1/62  
 [50] Field of Search 250/71, 80;  
 117/33.5, 313/92 PH

**ABSTRACT:** A plural color cathodoluminescent screen for use in a cathode-ray tube wherein at least two layers of light-emitting phosphors have therebetween a separation layer of electrically conductive oxide material that is substantially translucent to electromagnetic radiation and substantially opaque to the penetration of electron beams of predetermined velocity. The screen includes a nucleation to achieve the uniform disposition of an oxidizable metal which when substantially heated forms the metallic oxide of the separation layer.



PATENTED SEP 7 1971

3,603,792



Fig. 1



Fig. 2



Fig. 3

INVENTORS  
ANTHONY V. GALLARO,  
WALTER F. KAZUK &  
KENNETH SPEIGEL

BY *Donald R. Castle*  
ATTORNEY

## LUMINESCENT SCREEN HAVING A SEPARATION MEDIUM THEREIN

### CROSS-REFERENCE TO RELATED APPLICATIONS

This application is a divisional application of Ser. No. 634,724, filed Apr. 28, 1967, now U.S. Pat. No. 3,526,527, which is assigned to the assignee of the present invention. This divisional application contains matter disclosed but not claimed in another application Ser. No. 853,083 filed concurrently herewith, which application is also a division of Ser. No. 634,724, now U.S. Pat. No. 3,526,527.

### BACKGROUND OF THE INVENTION

This invention relates to beam penetration types of cathodoluminescent color screens and more particularly to screens having different layers of color-emitting phosphors excited by electron beams of differing velocities.

It is common in beam penetration multilayer cathodoluminescent screens to utilize a separation layer between adjacent phosphor layers to limit the penetration of electron beams of predetermined velocity. Conventional electron energy absorbing materials used in such separation structures include depositions of metals such as aluminum and magnesium and of nonconductive substances, as for example, mica and silicon dioxide. Certain disadvantages have been noted in screens employing such separation or barrier layers, for instance, metal deposits of specific thicknesses sufficient to control the penetration by electron beams of predetermined velocities usually exhibit a degree of opacity which limits translucency to electromagnetic radiation. On the other hand, nonconductive silicon dioxide which is substantially translucent to light energy, in addition to being difficult to uniformly deposit, manifests and undesirable dielectric property which momentarily retains an electron charge at the point of beam impingement. For example, the electron charge retention characteristic of the silicon dioxide layer slightly prolongs the excitation of the phosphor distal to the beam source and temporarily imparts color impurity to the color emission of the lower velocity excitable phosphor proximal to the beam source.

### OBJECTS AND SUMMARY OF THE INVENTION

It is an object of the invention to reduce the aforementioned disadvantages and provide an improved beam penetration type of cathodoluminescent screen.

Another object is to provide a beam penetration screen that exhibits improved color purity of the low velocity beam excited color emission.

A further object is the provision of a beam penetration screen having a separation layer therein of improved uniformity.

The foregoing objects are achieved in one aspect of the invention by the provision of a cathodoluminescent screen having therein at least two layers of energy emitting phosphor materials with a uniform separation layer disposed therebetween. Such separation layer is of an electrical conductive oxide substance that is nondeleterious to the adjacent phosphor materials while exhibiting opacity to a predetermined level of discrete phosphor excitation energy and translucency to electromagnetic radiation. A nucleate of metal molecules dispersed over a first phosphor material enhances the deposition of a uniform coating of an oxidizable metal thereover. The application of heat to the partial screen structure volatilizes the heat decomposable material and oxidizes the metal coating to form the aforementioned separation layer. The second phosphor material is applied thereover.

### BRIEF DESCRIPTION OF THE DRAWING

FIG. 1 is a cross-sectional view illustrating a partially formed cathodoluminescent screen structure;

FIG. 2 is a cross-sectional view showing the screen structure of FIG. 1 after the baking step in screen processing; and

FIG. 3 is a fragmentary cross-sectional view of a cathode-ray tube wherein the screen structure of the invention is formed on the inner surface of the viewing panel.

### DESCRIPTION OF THE PREFERRED EMBODIMENT

For a better understanding of the present invention, together with other and further objects, advantages and capabilities thereof, reference is made to the following specification and appended claims in connection with the aforescribed drawing.

With reference to the figures, there is shown a partially formed luminescent screen structure 11 which is formed on a substantially transparent support medium 13 such as a glass substrate or the inner surface of a cathode ray tube face plate. The screen utilizes a plurality of phosphors, of which at least one is responsive to electron excitation. Additionally, a screen of this type may also include one or more phosphors that are responsive to electromagnetic radiation emitted by a related electron responsive phosphor. The process of forming the screen comprises the application of a layer of a first phosphor material 15 which is substantially translucent and capable of energy emission upon excitation. This phosphor is disposed on the support medium by one of several conventional techniques such as for example by the settling of phosphor through a liquid cushion. Due to the range of phosphor particle sizes comprising the first phosphor layer, a somewhat roughened surface results. It is important that the separation or barrier layer 25, which is subsequently formed thereover, has a uniform thickness; therefore, a layer of a heat decomposable material is applied in a conventional manner thereon to fill in the rough topography of the phosphor layer and provide a smooth surface thereover. Suitable heat decomposable materials may be lacquer solutions such as methyl methacrylate dissolved in toluene which is appropriate for spray application or nitrocellulose dissolved in amyl acetate which is suitable for float-type application. Upon drying, the lacquer film provides a smooth base on which the separation layer 25 is formed.

It has been found that a nucleation applied in the form of a dispersion of metal molecules enhances the adherence and uniform deposition of a compatible metal disposed thereover. The nucleated material 19, being a very thin dispersion or molecular film, provides microscopic "islands" which promote uniform adherence of the sequentially applied compatible coating of oxidizable metal 21 vaporized thereon.

Heating of the screen support medium and the aforescribed partially formed screen thereon is consummated at a time-temperature relationship that is not deleterious to the phosphor materials therein, but sufficient to volatilize and remove the heat decomposable material and convert the oxidizable metal to the oxide forming the separation layer 25. The metal oxide thus formed exhibits electrical conductivity, opacity to discrete phosphor excitation energy of a substantially predetermined level and translucency to electromagnetic radiation impinged thereon. As used herein, the designation "electromagnetic radiation" is intended to include the scope of the electromagnetic spectrum extending from gamma rays through infrared radiation. FIG. 2 illustrated the partial screen structure 11' after heating, which embodies the first phosphor and the separation layer of oxidized metal. Subsequently, a second phosphor material, capable of energy emission upon excitation, is disposed upon the separation layer by a technique conventional to the art.

In greater detail, a luminescent screen such as a cathodoluminescent screen having at least two electron responsive phosphors therein, as utilized in a plural color cathode ray tube, will be described along with a process for fabricating the same. The aforescribed process as shown in FIGS. 1 and 2 is likewise applicable in this instance for disposing the screen directly on the face panel surface of the tube.

With reference to FIG. 3, a cathode ray tube 31 is partially shown wherein means 35 for generating electron beams of predetermined velocities is shown. This source of beams com-

prises one or more electron guns oriented in spaced relationship to the improved beam penetration-type cathodoluminescent screen 39 which is formed on the inner surface of the tube face panel 13'. When a single gun beam source is employed, anode switching means is utilized to provide beams of differing velocities, whereas in a plural gun source, separate guns emanate low and high velocity beams respectively.

The first disposed phosphor layer 15' is in the form of an electron responsive color-emitting material such as the E.I.A. P-1 phosphor ( $Zn_2SiO_4:Mn$ ) which is a green-emitting medium persistence material. This phosphor is disposed on the panel at a density range, in this instance, of approximately 3 to 5 mg/cm<sup>2</sup>. Next, one of the aforementioned lacquer materials is spray disposed thereover and the nucleate dispersed by vaporization thereon. The dispersion of the nucleate is of a minute thickness not deleterious to the translucency of the subsequently formed separation layer. It has been discovered that a suitable nucleating material is in the form of a metallic element requiring a vaporization temperature of at least 500° C. to consummate the evaporation thereof at a pressure of 10<sup>14</sup> torr. Such metals include, for example, silver, tin, aluminum, and chromium. In this embodiment, a molecular dispersion of vaporized aluminum is utilized as the nucleating material.

Upon the nucleate, a uniform coating of at least one metallic element selected from Groups 1b to 4a inclusive of Periods IV and V of the Periodic Table of Elements is vaporized thereon. Elements in these designations have oxide forms that are electrically conductive, translucent to light energy and exhibit opacity to electron beams of predetermined velocities in relationship to the thickness of the oxide layer. One of the Period V elements is, for example, cadmium which is utilized as the evaporated metallic coating in this embodiment of the invention. The partially formed screen structure is heated to approximately 400° C. for a time period of about 45 minutes to remove the lacquer material by volatilization and convert the cadmium deposition to a continuous separation layer 25' and convert the cadmium deposition to a continuous separation layer 25' of electrically conductive cadmium oxide having a uniformity of thickness. In this instance, the thickness of the cadmium oxide is in the order of 900 Angstroms. The temperature of the heating is not deleterious to the P-1 phosphor contained in the screen. It will be noted that the cadmium oxide separation layer 25' extends partially on the wall of the tube due to the deposition of the basic materials; i.e., the lacquer being spray applied and the nucleated aluminum and cadmium being vaporized thereon.

A layer of a second electron responsive phosphor 27 such as E.I.A. P-22 R.E.Red ( $YVO_4:Eu$ ), a high efficiency red-emitting phosphor, is disposed in a conventional manner over the separation layer and is of a substantially uniform density within the range of approximately 1 to 3 mg/cm<sup>2</sup>. A conductive coating 37, such as aquadag applied to the funnel and neck portions of the tube, makes contact with the separation layer and provides the anode connective path. The cathodoluminescent screen so described provides an outstanding two color display, the specific phosphors being excited to color emission by electron beams of different velocities.

The low velocity electron beam 41, emanating from the beam generating source, is in this instance in the order of 6 kv. which excites the second or red-emitting phosphor 27 to bright color emission but has insufficient velocity to penetrate through the separation layer 25'. The luminous red emission thus produced traverses the optically translucent separation layer and the optically translucent P-1 phosphor to be visible as a bright red display to the observer viewing the face panel of the tube.

The high velocity beam 43 being, for example, in the order of 12 kv. excites the second or red-emitting phosphor and is of sufficient velocity to traverse the separation layer and excite

the first or green-emitting phosphor layer disposed on the face panel. Since, in this instance, it is desired that a green color be observed as a result of high velocity beam excitation, the first or green-emitting phosphor is disposed in an amount to insure predominance of the green emission over the red therebeneath when the two are coincidentally excited by a common beam. Thus, from the viewpoint of the observer, distinct bright red and bright green displays are produced by the low and high velocity beams respectively. If the two beams are generated and directed to simultaneously impinge upon contiguous screen areas, a bright complementary color combination results.

The composition of the substantially translucent and electrically conductive separation or barrier layer 25' is important as the conductivity characteristic thereof readily dissipates the beam impingement charge thereon and provides two-fold results not evidenced in nonconductive capacitance prone separators. Firstly, the spot size of the red and green color emissions are both of a size smaller due to the absence of the capacitance characteristic which normally tends to retain some of the electron charge at the point of beam impingement causing the beam spot to "bloom". Secondly, when a beam is switched from high velocity to low velocity operation, the electron charge at the point of impingement is dissipated so that there is no deleterious carryover of green excitation and emission to momentarily lend color impurity to the desired red emission from the second phosphor layer. Hence the beneficial characteristics of the cadmium oxide separation layer relate to its translucency which readily conveys the luminescent brightness of the second phosphor layer, and to its conductivity which improves small spot size of both phosphor emissions and color purity of the luminescence emitted by the second or red-emitting phosphor.

Thus, there is provided a beam penetration type of cathodoluminescent screen that exhibits improved brightness and color purity heretofore sought but not previously evidenced in the beam penetration type of screen. The metallic nucleation advantageously facilitates the uniform deposition of the improved separation layer and expedites fabrication of the subject screen.

While there has been shown and described what is at present considered the preferred embodiment of the invention, it will be obvious to those skilled in the art that various changes and modifications may be made therein without departing from the scope of the invention as defined by the appended claims.

We claim:

1. In a cathodoluminescent screen having at least first and second layers of energy-emitting phosphor materials therein, at least one separation medium disposed therebetween to effect a barrier for a predetermined level of at least one type of energy, said medium comprising:

a continuous and uniform barrier layer of an electrical conductive oxide of at least one metallic element selected from Groups 1b to 4a inclusive of Periods IV and V of the Periodic Table, said oxide substance being nondeleterious to said phosphor materials and exhibiting opacity to discrete phosphor excitation energy of a substantially predetermined level and translucency to electromagnetic radiation impinged thereon; and

a nucleate of metal molecules of at least one substance selected from the group consisting of silver, tin, aluminum, and chromium, said nucleate being dispersed as islands over said first layer of said phosphor materials.

2. A luminescent screen separation medium according to Claim 1 wherein said conductive substance comprises cadmium oxide material.

3. A luminescent screen separation medium according to Claim 2 wherein the thickness of said cadmium oxide layer is in the order to 900 Angstroms.

UNITED STATES PATENT OFFICE  
CERTIFICATE OF CORRECTION

Patent No. 3,603,792 Dated September 7, 1971

Inventor(s) Anthony V. Gallaro, Walter F. Kazuk, Kenneth Speigel

It is certified that error appears in the above-identified patent and that said Letters Patent are hereby corrected as shown below:

In the Abstract, lines 8 & 9 (substantially) should read - - (subsequently) - - .

Column 1, line 35 of the specification (and) should read - - (an) - - .

Column 3, line 21 of the specification ( $10^{14}$ ) should read - - ( $10^{-4}$ )

Column 3, lines 39-40 of the specification, second instance, - - (and convert the cadmium deposition to a continuous separation layer 25') should be deleted - - .

Signed and sealed this 21st day OF March 1972.

(SEAL)

Attest:

EDWARD M.FLETCHER, JR.  
Attesting Officer

ROBERT GOTTSCHALK  
Commissioner of Patents